

J. RENTON.

Making Iron direct from Ore.

No. 11,838.

Patented Oct. 24, 1854.



# UNITED STATES PATENT OFFICE.

JAMES RENTON, OF CLEVELAND, OHIO.

## IMPROVEMENT IN MAKING WROUGHT-IRON DIRECT FROM THE ORE.

Specification forming part of Letters Patent No. 11,838, dated October 24, 1854.

*To all whom it may concern:*

Be it known that I, JAMES RENTON, of Cleveland, Ohio, have invented a new and useful Improvement in Furnaces for Making Iron Direct from the Ore, of which the following is a full, clear, and exact description, reference being had to the accompanying drawings, making part of this specification, in which—

Figure 1 is a perspective view of the improved furnace; Fig. 2 a longitudinal and Fig. 3 a cross section thereof; and Fig. 4 another cross-section at *a a*, Fig. 2.

The same letters indicate the same parts in all the figures.

My present invention is of an improvement in the process of making iron direct from the ore described in the patent granted to Alexander Dickinson, bearing date the 22d of July, 1850, and to myself bearing date the 23d of December, 1851, which process consists in deoxidizing the ore in a close chamber, so combined with the puddling-furnace that the ore which is deoxidized by the waste heat of the puddling-furnace without the products of combustion coming in contact with the ore shall be delivered directly onto the puddling-bottom from the deoxidizing-chamber without exposure to the atmosphere; and my said invention consists in combining, with a puddling-furnace and close deoxidizing-chamber, the introduction of a blast of atmospheric air, heated or cold, into the puddling-chamber, and discharged directly onto the ore after it has been delivered from the deoxidizing-chamber onto the puddling-bottom, and during the operation of deoxidizing, to facilitate the discharge of the carbon, and increasing the heat by inflaming the combustible evolved.

In the accompanying drawings, *a* represents the series of vertical deoxidizing-chambers, in which the ore is charged with carbon, to be deoxidized by the heated products of combustion which pass through a series of flues, *b*, at the sides of the chambers. These chambers *a* are placed over the rear end of the bottom *c* of a puddling-furnace, *d*, so that when the ore is deoxidized it is discharged from the deoxidizing-chambers onto the pud-

dling-bottom, where the iron is puddled and balled.

The puddling or reverberatory furnace consists, as usual, of a fire-chamber, *e*, with ash-pit *f* and grate *g*, a bridge, *i*, and roof *j* to reverberate the flame onto the iron on the bottom in the process of preparation. In the roof, at *k*, there is a series of apertures or tuyeres ranged across the furnace and communicating with a pipe, *l*, with two branches, *m m*—one on each side—and passing through the flues *b*, and thence connected with a suitable blowing apparatus. The blast forced in from the blower in passing through the branch pipes *m m* is heated, and in the heated state is blown in jets directly through the flame onto the iron on the puddling-bottom, by means of which the ore is more readily brought to the required condition for balling, to be worked into blooms by the usual means. After the iron has been properly treated in the puddling-furnace it may be, if desired, discharged through a door, *n*, into a refinery, *o*, placed at the side of the puddling furnace.

Instead of discharging the jets of air through tuyeres in the roof, they may be placed at the sides and inclined, although I prefer placing them in the roof; and instead of heating the air by passing the pipes through the flues, they may be carried through or along the side walls of the puddling-furnace, or around the fire-chamber, or in any other suitable or known manner of heating a blast, and, if desired, the air may be blown onto the iron in the cold state, although I prefer to have it heated.

I do not wish to be understood as limiting myself to the use of a puddling-furnace of the construction herein specified; nor of a deoxidizing apparatus such as herein specified; nor to the arrangement for delivering the ore from the deoxidizing-chamber onto the puddling-bottom; nor, finally, to the kind or arrangement of the apparatus, as these may be varied at pleasure so long as they are suited to the purpose contemplated.

I do not wish to be understood as making claim to the combination of the deoxidizing apparatus with the puddling-furnace to discharge the deoxidized ore directly onto the

puddling-bottom, as this has already been secured by Letters Patent, as before specified.

What I do claim as my invention, and desire to secure by Letters Patent, is—

Combining with the combined deoxidizing apparatus and puddling-furnace, as described, the employment of a blast or blasts to be forced onto the deoxidized ore on the

hearth or hearths, substantially as specified, to aid in decarbonizing the ore and increasing the heat; as specified.

JAS. RENTON.

Witnesses:

JAMES A. BRIGGS,  
W. H. BURRIDGE.